

1

3,824,135

## COPPER BASE ALLOYS

Michael J. Pryor, Woodbridge, Stanley Shapiro, New Haven, and Richard D. Lanam, Hamden, Conn., assignors to Olin Corporation  
No Drawing. Filed June 14, 1973, Ser. No. 369,914  
Int. Cl. C22c 9/06; C22f 1/08  
U.S. Cl. 148—32.5

6 Claims

### ABSTRACT OF THE DISCLOSURE

The disclosure teaches novel copper base alloys having improved toughness and outstanding resistance to stress corrosion. The copper alloys contain, in weight percentages, from 15 to 30% nickel, from 15 to 30% manganese, an element selected from the group consisting of aluminum from 0.01 to 5%, magnesium from 0.01 to 5%, boron from 0.001 to 0.1%, zinc from 0.1 to 3.5%, tin from 0.01 to 3%, zirconium from 0.01 to 2%, titanium from 0.01 to 2%, chromium from 0.01 to 1%, iron from 0.1 to 5%, cobalt from 0.05 to 1%, and mixtures thereof, together with 0.005 to 0.1% of an element selected from the group consisting of arsenic and antimony, and mixtures thereof.

### BACKGROUND OF THE INVENTION

Copper base alloys are known which contain relatively large amounts of nickel and manganese. Alloys of this type are highly desirable since they are capable of attaining yield strengths in excess of 200 k.s.i. upon aging. In addition, these alloys appear to have reasonable processing qualities and in particular are not quench sensitive.

The presence of a marked aging response to obtain high strengths in copper-nickel-manganese alloys is known. It has been found that different types of precipitation reactions may occur in this alloy system, depending on the aging temperature. For example, aging at a low temperature, such as 350° C., yields a cellular precipitate which nucleates at the grain boundaries and with time grows throughout the entire grain. The cellular precipitate consists of adjacent lamellae of a manganese-nickel rich phase and the copper-rich solid solution. Aging at higher temperatures, such as 450° C., yields mainly finely dispersed, spherical precipitates of the manganese-nickel rich phase within the grains and only a small amount of the cellular precipitate at the grain boundaries.

However, in any event, the presence of a cellular precipitate at grain boundaries is generally found to have deleterious effects on alloy properties, such as fracture toughness and stress corrosion resistance. This is indeed found to be the case in these alloys and is a significant factor in the limited commercial success of these alloys heretofore.

Generally, the copper base alloys used in springs and similar applications rely upon extensive cold work in order to achieve high strengths, for example, greater than 150 k.s.i. 0.2% offset yield strength. However, such extensive cold work imposes severe limitations on the subsequent formability of the alloys.

While known copper-2% beryllium age-hardenable alloys achieve yield strengths in the 150 to 200 k.s.i. range, have good formability in the un-aged condition, and exhibit good performance under stress corrosion conditions, such alloys are characterized as expensive, quench sensitive, and difficult or even dangerous to cast, thus exhibiting difficult processing properties. In contrast, the age-hardenable Cu-Ni-Mn alloys are relatively inexpensive, are not quench sensitive, and are characterized by favorable processing properties, such as being well adapted to hot or cold rolling. However, such alloys of the prior art have been inadequate with respect to toughness and par-

2

ticularly with respect to resistance to stress corrosion for especially demanding uses, such as in springs likely to be exposed to a corrosive atmosphere under stress. While significant improvement in these properties was attained in the alloys described in U.S. Pat. 3,712,837, a more beneficial combination of properties remained desirable, particularly with respect to increased resistance to stress corrosion.

Accordingly, it has been highly desirable to develop an alloy within the copper-manganese-nickel alloy system which has increased fracture toughness in combination with significantly improved stress corrosion resistance qualities.

Accordingly, it is a principal object of the present invention to develop an improved copper base alloy containing relatively large amounts of nickel and manganese.

It is an additional object of the present invention to develop an alloy as aforesaid which is capable of obtaining yield strengths in excess of 200 k.s.i. upon aging.

It is a still further object of the present invention to develop an alloy as aforesaid which is readily processed commercially and which is characterized by improved fracture toughness.

It is a still further object of the present invention to provide a copper base alloy with excellent stress corrosion resistance, good ductility, toughness and high yield strength characteristics.

Further objects and advantages of the present invention will appear from the ensuing discussion.

### SUMMARY OF THE INVENTION

In accordance with the present invention, it has now been found that the foregoing objects and advantages may be readily obtained.

The alloy of the present invention consists essentially of from 15 to 30% nickel, from 15 to 30% manganese, and an element selected from the group consisting of aluminum from 0.01 to 5%, magnesium from 0.01 to 5%, boron from 0.001 to 0.1%, zinc from 0.1 to 3.5%, tin from 0.01 to 3%, zirconium from 0.01 to 2%, titanium from 0.01 to 2%, chromium from 0.01 to 1%, iron from 0.1% to 5%, cobalt from 0.05 to 1%, and mixtures thereof, together with 0.005 to 0.1% of an element selected from the group consisting of arsenic, antimony, and mixtures thereof, with the balance essentially copper wherein the nickel to manganese ratio is at least 0.75 and preferably 1.0 or higher.

### DETAILED DESCRIPTION

In accordance with the present invention, the foregoing alloy has been found to obtain surprisingly improved fracture toughness while retaining the excellent strength characteristics of this alloy system.

This enables the attainment of several significant advantages. The alloy of the present invention is an excellent lower priced replacement for beryllium-copper, with increased fracture toughness. The alloy of the present invention achieves levels of fracture toughness approaching high alloy steels which are limited in applicability by poor corrosion resistance. The alloys of the present invention are superior to maraging steels in marine environments since the alloys of the present invention are not susceptible to hydrogen embrittlement. In addition, the alloys of the present invention are characterized by excellent stress corrosion resistance.

In accordance with the present invention, the instant alloys contain from 15 to 30% nickel, and from 15 to 30% manganese. Preferably, both the nickel and manganese contents should range from 15 to 25%. The nickel to manganese ratio must be at least 0.75 and preferably 1.0 or higher.

The nickel and manganese contents have an effect on aging response, yield strength and workability of the alloys. The lower the manganese and nickel content, the slower the aging response and lower the maximum yield strength obtainable upon aging, especially below 15% nickel and manganese. On the other hand, increasing the amount of nickel and manganese has deleterious effects on the workability of the alloys during processing, especially over 30% each of nickel and manganese.

As indicated hereinabove, the preferred nickel to manganese ratio is 1.0 or higher. The maximum aging response is obtained for a given amount of nickel and manganese when the nickel to manganese ratio is about 1.0. If the ratio is less than 1.0, an excess of manganese exists which can have adverse effects on the stress corrosion resistance of the alloy. A ratio greater than about 1.5 generally does not provide sufficiently improved results over a ratio of about 1.0 to justify the higher cost of the nickel.

In addition to the foregoing, the alloy of the present invention contains an element selected from the group consisting of aluminum in an amount from 0.01 to 5.0%, magnesium from 0.01 to 5.0%, boron from 0.001 to 0.1% zinc from 0.1 to 3.5%, tin from 0.01 to 3%, zirconium from 0.01 to 2%, titanium from 0.01 to 2%, chromium from 0.01 to 1%, iron from 0.1 to 5%, cobalt from 0.05 to 1%, and mixtures thereof.

Aluminum, magnesium, and boron act as deoxidizers and assist in the melting of the alloys. Aluminum is the preferred addition since it tends to form a protective oxide coating during melting. When aluminum is used as a deoxidant only, it should be added in an amount from 0.01 to 0.75%, and similarly for magnesium. Furthermore, the aluminum and magnesium may be used as advantageous alloying additions in amounts greater than 0.6% for increased corrosion resistance and fracture toughness. The aluminum when used at the higher levels, also tends to modify the cellular precipitate at the grain boundaries.

When zinc is an added component, it should be present in an amount from 0.1 to 3.5%. Increased amounts of zinc over 3.5% given rise to a decrease in the stress corrosion resistance and fracture toughness. The zinc addition tends to control the grain size, reduce the cellular precipitate at the grain boundaries, alter the morphology of the inclusions, promote sound castings and increase the aging response of the alloy. It is most surprising that so many advantages may be realized from a single alloying addition. The grain size control may be attributed to a fine dispersoid which is present in the zinc containing alloys. The increased aging response is due to an increase in the growth rate of the precipitate. The preferred zinc content is from 1 to 3%.

In addition to the foregoing, several additives are particularly advantageous. Tin is a particularly desirable additive in an amount from 0.01 to 3% and preferably from 0.5 to 2.0%. Tin tends to alter the morphology of the cellular precipitate at the grain boundary.

Zirconium and/or titanium are preferred alloying additions in amounts 0.01 to 2.0% each, and preferably from 0.15 to 0.30% each. These elements tend to effect desirable changes in the morphology and chemistry of inclusions and in the morphology of cellular precipitate at grain boundaries.

In addition, chromium is a desirable addition in an amount from 0.01 to 1.0%, and preferably from 0.15 to 0.30%. Chromium tends to control the grain size and change the morphology and chemistry of inclusions.

Additional desirable alloying additions are cobalt and/or iron. These elements are desirable for providing desired control of grain size. The cobalt may be employed in an amount from 0.05 to 1.0% and preferably from 0.2 to 0.5%, and the iron from 0.1 to 5% and preferably from 0.5 to 1.0%.

The advantageous combination of outstanding resist-

ance to stress corrosion, physical properties such as to enable excellent performance in demanding uses, and desirable formability qualities in the alloys is attained with certainty in accordance with this invention through the further addition of a small but essential proportion of arsenic or antimony or mixture thereof within the range of 0.005 to 0.1% by weight. Such addition has been found to assure the proper control of grain size and the desired dispersion of fine precipitate mostly throughout the interior of the grains, which have been indicated as essential for the desired alloy qualities and performance.

It is noteworthy that such effects of the arsenic and antimony additions differ essentially from those customarily obtained in single phase copper-base alloys. In the latter, the additions have customarily been made to reduce dezincification. If the alloy is not single phase, the general experience has been that no beneficial effect from the addition is found. The alloys of the present invention comprise an age hardening system. They are polyphase in the final heat treated condition. It is, therefore, quite surprising that the addition of arsenic and/or antimony would result in the improved stress corrosion performance noted for these alloys in both industrial and marine environments.

However, single phase copper base alloys containing arsenic and antimony are known to be hot short, exhibiting such limited hot rollability that they must generally be subjected only to cold rolling. In contrast, the alloys of the present invention are hot rollable and are single phase in the hot working temperature range. It is quite surprising that a single phase copper base alloy containing either arsenic and/or antimony in these amounts is hot rollable.

The casting of the alloy of the present invention is not particularly significant. Any convenient method of casting may be employed. Pouring temperatures in the range of about 1000 to 1200° C. are preferably employed, with an optimum pouring temperature in the range of 1050 to 1100° C. The arsenic and/or antimony additions should be as a master alloy prior to pouring, for convenience due to the toxicity of these materials.

Generally, the alloy of the present invention is processed by breakdown of ingot into strip using a hot rolling operation followed by cold rolling and annealing cycles to reach final gage. Preferred properties are obtained using an aging treatment.

The starting hot rolling temperature should be in the range of 700 to 900° C., and preferably 750 to 850° C. The cooling rate from hot rolling should preferably be in excess of 25° C. per hour down to 300° C. in order to avoid precipitation of manganese-nickel rich phases. The cooling rate after 300° C. is not significant. The alloy is capable of cold rolling reductions in excess of 90%, but the cold rolling reduction should preferably be between 50 and 80% in order to control the grain size.

It has been found that an average grain size less than 0.005 mm. is necessary in order to provide optimum stress corrosion resistance. Generally, an average grain size in the alloys of the present invention of less than 0.003 mm. is readily obtained. An average grain size of this order can be obtained by control of the cold rolling reduction, annealing times and annealing temperatures. In general, anneal-temperatures in the range of 550 to 900° C. for at least one minute can give the required grain size, with 10 hours being the practical upper limit and 2 hours being the preferred upper limit. It is preferred to anneal for from five minutes to 2 hours.

After annealing, the material is cooled in excess of 25° C. per hour down to 300° C., as indicated above, and the cold rolling and annealing cycles repeated as desired depending on gage requirements. Generally, from two to four cycles of cold rolling and annealing are preferred.

The present invention will be more readily understandable from a consideration of the following illustrative examples.

## EXAMPLE I

A 10 lb. ingot of an alloy containing 25.0 nickel, 17.0 manganese, 2.0 zinc, 0.5 aluminum, .04 antimony (Alloy A) and the balance copper was prepared in strip form in the following manner. The alloy was melted from elemental constituents except for the antimony which was added as a copper-antimony master alloy and chill cast from 1200° C. into a steel mold. The ingot was soaked

increasing the yield strength level at which the alloy can be used.

## EXAMPLE III

Example II was repeated for Alloy D except that the samples were cold worked 40 and 50% prior to aging. Alloy C was treated with 40% cold work prior to aging for comparison purposes. The data is shown in Table B below.

TABLE A  
Solution heat treat plus 25% cold work

| Alloy | Aging treatment    | 0.2% offset yield strength, k.s.i. | Tensile strength, k.s.i. | Percent elongation, inches | Time to failure—New Haven—days | Time to failure—Daytona—days |
|-------|--------------------|------------------------------------|--------------------------|----------------------------|--------------------------------|------------------------------|
| A     | 450° C. X3.5 hours | 168.0                              | 178.8                    | 6.5                        | 278                            | 140                          |
| A     | 450° C. X6.0 hours | 183.5                              | 192.5                    | 5.3                        | 69                             | 52                           |
| B     | 450° C. X5.0 hours | 156.1                              | 173.5                    | 10.0                       | 204                            | 4                            |
| B     | 450° C. X8.0 hours | 169.3                              | 185.0                    | 8.8                        | 59                             | 9                            |
| C     | 450° C. X4.0 hours | 158.3                              | 177.5                    | 10.3                       | 81                             | 12                           |
| C     | 450° C. X8.0 hours | 182.0                              | 198.0                    | 6.5                        | 16                             | 2                            |
| D     | 450° C. X3.5 hours | 168.3                              | 179.5                    | 7.0                        | 309                            | 143                          |
| D     | 450° C. X6.0 hours | 184.7                              | 196.5                    | 7.0                        | 81                             | 39                           |

TABLE B  
Solution heat treat plus 40% cold work and 50% cold work

| Alloy and condition | Aging treatment    | 0.2% offset yield strength, k.s.i. | Tensile strength, k.s.i. | Percent elongation, inches | Time to failure—New Haven—days | Time to failure—Daytona—days |
|---------------------|--------------------|------------------------------------|--------------------------|----------------------------|--------------------------------|------------------------------|
| 40% cold work:      |                    |                                    |                          |                            |                                |                              |
| C                   | 450° C. X4.0 hours | 168.0                              | 185.0                    | 6.0                        | 52                             | 26                           |
| D                   | 450° C. X8.0 hours | 185.4                              | 195.0                    | 2.0                        | 1>180                          | 1>120                        |
| 50% cold work: D    | 450° C. X8.0 hours | 188.3                              | 200.3                    | 4.0                        | 1>180                          | 1>120                        |

<sup>1</sup> Samples still in test.

at 845° C. and hot rolled from 1.5" to .250". The hot rolled plate was cold rolled to 0.100" and annealed at 600° C. for 30 minutes. The plate was cold rolled 60% to .040" and annealed at 600° C. for 30 minutes. The material was cold rolled 25% to a final gauge of 0.030". Samples of the 25% cold rolled strip at 0.030" were formed into 90° U-bends by bending a strip 6" long by 1/2" wide around a mandrel so that it permanently forms a 90° bend, and transverse tensile samples were fabricated. The U-bends and tensile specimens were aged for various times at 450° C. After the aging treatment, the U-bends were sprung into jigs which hold the ends of the samples 1" apart. The resulting tensile properties and stress corrosion results are presented in Table A. The tensile results are the average of two transverse samples; the stress corrosion results the average of five U-bends. New Haven, Connecticut, is an industrial environment and Daytona Beach, Florida, a marine environment. Data for a copper-25 nickel-17 manganese-2 zinc alloy (Alloy B) and copper-20 nickel-20 manganese-0.5 Al (Alloy C) are also presented for comparison purposes. These were processed in a similar manner to the antimony containing alloy.

## EXAMPLE II

An alloy containing 25 nickel, 17 manganese, 2 zinc, 0.5 aluminum, 0.04 arsenic (Alloy D) and balance copper was prepared in strip form by a similar practice to that described above. The tensile properties and stress corrosion results are also listed in Table A.

The improvement in the stress corrosion life becomes even more evident when the times to failure in New Haven and Daytona Beach are examined in terms of yield strength. The effect of the antimony and arsenic additions in both New Haven and Daytona Beach is to increase the time to failure at a given yield strength, thus

40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855

6. An alloy according to Claim 1 containing aluminum in an amount from 0.01 to 5.0%, zinc from 0.1 to 3.5% and arsenic from 0.005 to 0.1%.

**References Cited**

**UNITED STATES PATENTS**

|           |         |                |            |
|-----------|---------|----------------|------------|
| 3,712,837 | 1/1973  | Shapiro et al. | 148—11.5 R |
| 3,402,043 | 9/1968  | Smith          | 75—157.5   |
| 2,234,552 | 3/1941  | Dean et al.    | 75—159     |
| 2,061,921 | 11/1936 | Roath          | 75—157.5   |

**FOREIGN PATENTS**

|             |         |               |          |
|-------------|---------|---------------|----------|
| 577,597     | 5/1946  | Great Britain | 75—159   |
| 578,223     | 6/1946  | Great Britain | 75—159   |
| 1,092,218   | 11/1960 | Germany       | 75—159   |
| 5 1,183,692 | 12/1964 | Germany       | 75—157.5 |
| 24,220      | 10/1964 | Japan         | 75—159   |

CHARLES N. LOVELL, Primary Examiner

U.S. Cl. X.R.

75—153, 154, 157 159; 148—11.5; 148—12.7